

# UNITED STATES PATENT OFFICE.

OTTO RÖHM, OF DARMSTADT, GERMANY.

## PROCESS FOR PRODUCING LEATHER WITH THE ASSISTANCE OF IRON SALTS.

1,364,317.

Specification of Letters Patent.

Patented Jan. 4, 1921.

No Drawing. Application filed March 10, 1917, Serial No. 154,034. Renewed May 28, 1920. Serial No. 385,065.

To all whom it may concern:

Be it known that I, Otto RÖHM, a citizen of Germany, residing at No. 4-6 Weiterstädterstrasse, in the city of Darmstadt, 5 Grand Duchy of Hessa, German Empire, have invented an Improvement in Processes for Producing Leather with the Assistance of Iron Salts; and I do hereby declare that the following is a full, clear, and exact description of the same.

According to the process set forth in my patent application Serial No. 154,033, ferric iron salts are used to produce leather by allowing aldehyde, preferably formaldehyde, said iron salts being preferably basic ferric iron chlorid, to act on the skins. This iron and aldehyde tanning process can also be combined with a treatment of the skins with neutralizing or iron precipitating substances, such as ammonia, alkalis, alkaline salts or with phenols, naphthols, organic carbon acids, vegetable tanning substances, or with soaps, sulfids, polysulfids or the like.

Now it has been found that the advantages of a combined aldehyde and iron tanning process are also obtained if the aldehyde-tanning process is carried out simultaneously with, or even after, the neutralizing of the leather, subsequent to the metal tanning, has been effected. If the aldehyde treatment is carried out simultaneously with the neutralizing process the further advantage is obtained that the warping of the grain which otherwise occurs is avoided, 35 and a specially fine, intricate and very durable grain is obtained.

Example: 100 parts depilated skins are worked 1 to 2 hours with 200 parts water+5 parts of 40% formaldehyde solution+2 parts of sodium bicarbonate. The skins are then washed with water and with 2/3 basic ferric iron chlorid in doses of 10—20% until the desired quantity of iron has been taken up, all as set forth in my copending application above noted.

In carrying out this improved process, the skins treated as specified are subjected to a further treatment with 2% formaldehyde which is used simultaneously with the neutralizing process effected with 1 to 3% soda,

preferably sodium bicarbonate, according to the strength of the tanning extract.

Further advantages have been obtained when the tanning is carried out with a mixture of various metal salts. In doing so 55 leather is obtained having new properties. While common iron leather, for example, shrinks together in water of but 60° C., and a leather tanned with ferric iron salt and aldehyde shrinks at about 90° C., a mixed 60 tanning, firstly with chrome salt, and then with ferric iron salts, yields a leather which is stable when boiled and is also fuller and heavier than common chrome leather.

What I claim and desire to secure by 65 Letters Patent of the United States is:—

1. The process for producing leather, which consists in tanning the skins with ferric iron salts, followed by a neutralization with ferric iron compound precipitating 70 substances and a treatment with aldehydes.

2. The process for producing leather which consists in tanning the skins with basic ferric iron chlorid followed by a neutralization with ferric iron compound precipitating 75 substances and a treatment with aldehydes.

3. The process for producing leather which consists in tanning the skins with ferric iron salts followed by a neutralization 80 with alkalis and a treatment with aldehydes.

4. The process for producing leather which consists in tanning the skins with ferric iron salts followed by a neutralization 85 with sodium bicarbonate, and a treatment with aldehydes.

5. The process for producing leather which consists in tanning the skins with ferric iron salts followed by a neutralization 90 with iron compound precipitating substances and a treatment with formaldehyde.

6. The process for producing leather which consists in tanning with ferric iron salts followed by a neutralization with iron 95 compound precipitating substances and a simultaneous treatment with aldehydes.

7. The process for producing leather which consists in tanning the skins with basic ferric iron chlorid followed by a neu- 100

tralization with 1 to 3% sodium bicarbonate and a simultaneous treatment with 2% formaldehyde.

8. The process for producing leather which consists in tanning the skins with ferric iron salts and with other metal salts followed by a treatment with aldehydes.

9. The process for producing leather which consists in tanning the skins with chrome salts, then tanning said skins with ferric iron salts, followed by a treatment with aldehydes.

OTTO RÖHM.